

# United States Patent [19]

Kimura et al.

[11] 3,793,020

[45] Feb. 19, 1974

- [54] **PHOTOGRAPHIC SILVER HALIDE EMULSIONS SENSITIZED WITH BENZIMIDAZOLE CYANINE DYES**
- [75] Inventors: Shiro Kimura, Kanagawa; Yoshiyuki Nakazawa, Nakanuma; Akira Sato, Minami Ashigara; Yashuharu Nakamura, Ashigara-Kamigun, all of, Japan
- [73] Assignee: Fuji Photo Film Co., Ltd., Kanagawa, Japan
- [22] Filed: Sept. 1, 1972
- [21] Appl. No.: 285,694

#### Related U.S. Application Data

- [63] Continuation of Ser. No. 664,287, Aug. 30, 1967, abandoned.
- [30] **Foreign Application Priority Data**  
Aug. 30, 1966 Japan ..... 41-57141
- [52] U.S. Cl. .... 96/137, 260/240.6, 260/240.65  
[51] Int. Cl. .... G03c 1/18  
[58] **Field of Search** ..... 96/137

- [56] **References Cited**  
UNITED STATES PATENTS  
2,503,776 4/1950 Sprague ..... 96/137

2,945,763 7/1960 Jones ..... 96/137

*Primary Examiner*—J. Travis Brown  
*Attorney, Agent, or Firm*—Sughrue, Rothwell, Mion, Zinn & Macpeak

#### [57] ABSTRACT

A photographic silver halide emulsion having higher sensitivity and markedly reduced color staining incorporating a novel sensitizing dye represented by the general formula:



wherein each of groups V<sub>1</sub>, V<sub>2</sub>, W<sub>1</sub>, and W<sub>2</sub> is a hydrogen or halogen atom, each of groups R<sub>1</sub> and R<sub>2</sub> is a lower alkyl group, A is a group selected from polymethylene and alkylpolymethylene group, and n is an integer from 1 to 4.

**5 Claims, No Drawings**

**PHOTOGRAPHIC SILVER HALIDE EMULSIONS  
SENSITIZED WITH BENZIMIDAZOLE CYANINE  
DYES**

This is a continuation of application Ser. No. 664,287, filed Aug. 30, 1967, now abandoned and claiming priority from Aug. 30, 1966 based on Japanese Pat. application Ser. No. 357141/66.

**BACKGROUND OF THE INVENTION**

1. Field of the Invention

The present invention relates to photographic silver halide emulsions containing a novel sensitizing dye.

2. Description of the Prior Art

It is known in the techniques of producing photographic silver halide emulsions that by adding a sensitizing dye to the silver halide emulsion the spectral light-sensitivity range of the silver halide emulsion is enlarged, i.e., the emulsion is optically sensitized.

However, in general, photographic silver halide emulsions containing sensitizing dyes usually are accompanied by color staining caused by the remaining sensitizing dye, after the completion of photographic processings, such as developing, fixing, stabilizing and water-washing. Such color stains, after processing, reduce the whiteness of the finished printing paper in photographic printing paper and worsens the color hue of the image and has a bad influence on color reproduction in photographic color films.

Therefore, an object of this invention is to provide a photographic silver halide emulsion in which by employing an improved sensitizing dye, the formation of color stains is markedly reduced. Another object of this invention is to provide a photographic silver halide emulsion having a higher sensitivity than conventional silver halide emulsions.

**SUMMARY OF THE INVENTION**

The objects of this invention can be achieved by incorporating a novel sensitizing dye represented by the following general formula (A) in a photographic silver halide emulsion:



which is an asymmetrical benzimidazolocarbocyanine dye having a sulfoalkyl group as a substituent at the nitrogen atom of one nucleus and a carboxyalkyl group at the nitrogen atom of another nucleus, wherein  $V_1$ ,  $V_2$ ,  $W_1$  and  $W_2$ , which may be the same or different, each represents a hydrogen atom, or a halogen atom, such as a chlorine atom, a bromine atom, an iodine atom or a fluorine atom;  $R_1$  and  $R_2$ , which may be the same or different, each represents a lower alkyl group, such as, a methyl group, an ethyl group, an *n*-propyl group, or an *n*-butyl group;  $A$  represents a polymethylene group, such as, an ethylene group, a trimethylene group or a tetramethylene group or an alkylpolymethylene group, such as, a methyltrimethylene group; and  $n$  is an integer of from 1 to 4.

The sensitizing dye, asymmetrical benzimidazolocarbocyanine dye, may be prepared by a conventional condensation process. Hereinafter, general processes of preparing an intermediate product for the sensitizing dye used in this invention and of preparing the sensitizing dye itself will be described.

A quaternary salt of benzimidazolium, which is an intermediate product of the sensitizing dye of this invention, may be obtained by reacting a benzimidazole with

10  $\alpha$ -bromoacetic acid,  $\beta$ -bromopropionic acid,  $\beta$ -iodopropionic acid,  $\gamma$ -bromobutyric acid, and the like, but for preparing the pure benzimidazolium quaternary salt with a good yield, a benzimidazole is caused to react with an acid amide compound or a nitrile compound of the aforesaid carboxylic acid instead of reacting with the carboxylic acid to provide a quaternary salt, which is then hydrolyzed with a mineral acid such as hydrobromic acid to provide the quaternary salt of benzimidazolium having a carboxyalkyl group. By reacting the aforesaid quaternary salt with diphenylformamidine, an anilinovinyl intermediate product represented by the general formula (B) is prepared:



wherein  $V_1$ ,  $V_2$ ,  $R$  and  $n$  are as defined above in regard to general formula (A), and  $X$  represents an anion such as a chloride, bromide, iodide, or perchloride.

The anilinovinyl intermediate product (B) is caused to react with acetic anhydride in a suitable solvent, such as nitrobenzene, to provide an acetoanilidovinyl intermediate product, and by reacting the intermediate product thus prepared with a quaternary salt represented by the following general formula (C) in the presence of a suitable organic base, such as triethylamine or *N*-alkylpiperidine by adding the quaternary salt to the reaction solution, the benzimidazolocarbocyanine dye shown by formula (A) is obtained:



wherein  $W_1$ ,  $W_2$ ,  $R_2$ , and  $A$  are as defined above in regard to general formula (A).

As typical examples of the anilinovinyl intermediate product represented by general formula (B), there are illustrated the following two compounds (1) and (2):





(2)

The anilinovinyl intermediate shown by the above formula (1) may be prepared as follows:

A mixture of 4 g. of 1-γ-carboxypropyl-5,6-dichloro-3-ethyl-2-methylbenzimidazolium bromide and 4 g. of diphenylformamidine was heated to 160° C on an oil bath and after removing under reduced pressure the aniline thus formed, the reaction was continued for 1 hour more. After the end of the reaction, the crystal obtained was washed with acetone to provide 3.7 g. of the light-yellow crystal having a melting point of 220° C.

The anilinovinyl intermediate product shown by formula (2) may be also prepared by a similar process as used to prepare compound (1). The melting point thereof was 215° C.

Typical examples of sensitizing dyes used in this invention are as follows:



(I)



(II)



(III)



(IV)

The sensitizing dye shown by formula (I) may be prepared as follows:

4.7 g. of the intermediate product (2), 2-(β-anilinovinyl)-1-carboxymethyl-5,6-dichloro-3-ethylbenzimidazolium bromide was heated under refluxing for 15 minutes in a mixture of 2 ml. of acetic anhydride and 20 ml. of nitrobenzene. The resulting solution was mixed with 3.8 g. of anhydro-5,6-dichloro-1-ethyl-2-methyl-3-(3-sulfobutyl)-benzimidazolium hydroxide and 2 ml. of triethylamine and the mixture was heated under refluxing for 10 minutes. After cooling, ether was added to the product to precipitate the dye. The precipitate was washed with water and recrystallized from a mixed solution of methanol and chloroform to provide 1.2 g. of the crystals of the sensitizing dye (I) having a melting point of 238° C (decomposed). The spectral absorption maximum of the dye in methanol was 518 m.μ.

Sulfur analysis: calculated: 4.84%, Found: 4.61%.

Sensitizing dye (II) was also obtained by the same procedure as above. The melting point of the dye was 270° C (decomposed), and the spectral absorption maximum of the dye in methanol was 513 m.μ.

Sulfur analysis: calculated: 4.98%, Found: 4.73%.

Sensitizing dye (III) was also obtained by the same procedure. The melting point thereof was 284° C. (decomposed), and the spectral absorption maximum of the dye in methanol was 518 m.μ.

Sulfur analysis: calculated: 4.73%, Found: 4.65%.

Sensitizing dye (IV) was also obtained by the same procedure as in the case of preparing dye (I). The melting point thereof was 236° C. (decomposed), and the spectral absorption maximum of the dye in methanol was 518 m.μ.

Sulfur analysis: calculated: 4.84%, Found: 4.68%.

In the silver halide emulsion used in this invention may be used various silver salts, such as silver chloride, silver bromide, silver iodide, silver iodobromide, and the like.

In order to prepare the sensitized photographic silver halide emulsion of this invention, one or more of the sensitizing dyes may be incorporated into the photographic silver halide emulsion by a conventional method.

Since the concentration of the sensitizing dye in the emulsion may be in a range of from 1 to 150 mg. per one kg. of the emulsion, the concentration thereof may be varied in the wide range according to a desired effect.

The sensitizing dye used in this invention may be incorporated into a photographic silver halide emulsion which had been sensitized by physical reprocessing and chemical reprocessing.

Moreover, in the production of the photographic silver halide emulsion, there may be added to the emulsion by a conventional method additives such as a sensitizer, a stabilizer, a color toning agent, a hardening agent, a wetting agent, an anti-foggant, a plasticizer, a development accelerator, a coupler and a fluorescent whitening agent.

The photographic silver halide emulsion of this invention may be applied to a suitable support such as a glass plate, a cellulose derivative film, a synthetic resin film or a baryta paper.

The novel sensitizing dye used in this invention is a very useful sensitizer since when the sensitizing dye is incorporated into a photographic silver halide emul-

sion, it sensitizes spectrally the silver halide emulsion and, in particular, in the case of a gelatino silver halide emulsion it enlarges the spectral light-sensitive range of the emulsion. Furthermore, the sensitizing dye can also be used as a sensitizer for a photographic silver halide emulsion containing a hydrophilic colloid other than gelatin, such as agar agar, collodion, a water-soluble cellulose derivative, polyvinyl alcohol, etc., or other hydrophilic synthetic or natural resin.

When the photographic silver halide light-sensitive element having the silver halide emulsion layer containing the novel sensitizing dye of this invention is subjected to photographic processings, such as developing, fixing and water washing, coloring of the image-bearing layer by the remaining dye is very low and further, since the sensitizing dye has a low co-action to a compound having an anionic group, such as a surface active agent, color coupler and the like, the color sensitizing property of the dye is not affected by the presence of such an anionic compound.

#### EXAMPLE

A silver iodobromide emulsion (the mole ratio of AgI to AgBr was 7:93) or a silver chlorobromide emulsion (the mole ratio of AgBr to AgCl was 40:60) each containing the sensitizing dye of this invention was applied to a film base and dried. The film thus prepared was exposed to day light of 64 lux (5,400° K) through Fuji No. 3 Filter (made by Fuji Photo-Film Co.; passing light having wave lengths longer than 500 m.μ.) and developed. As the developer, one having the composition shown in Table 1 was used for the silver iodobromide emulsion layer and one having the composition shown in Table 2 was used for the silver chlorobromide emulsion layer. The results are shown in Table 3 and Table 4.

TABLE 1

|                        |          |
|------------------------|----------|
| N-Methyl-p-aminophenol | 20 g.    |
| Hydroquinone           | 5.0 g.   |
| Sodium Sulfite         | 100 g.   |
| Borax                  | 20 g.    |
| Water To Make          | 1000 ml. |

TABLE 2

|                                |          |
|--------------------------------|----------|
| N-methyl-p-Aminophenol Sulfate | 20 g.    |
| Hydroquinone                   | 40 g.    |
| Sodium Sulfite                 | 40 g.    |
| Sodium Carbonate (Anhydrous)   | 24 g.    |
| Potassium Bromide              | 1 g.     |
| Water To Make                  | 1000 ml. |

Filter, while defining the sensitivity of the silver iodobromide emulsion, containing no novel sensitizing dye of this invention, to be 100.

TABLE 4

| Test No. | Sensitizing Dye | Amount (mg. mole/kg. emulsion) | Emulsion | Density of Color Stain |
|----------|-----------------|--------------------------------|----------|------------------------|
| 1        | (I)             | 0.09                           | AgBr-Cl  | 0.02                   |
| 2        | (V)*            | 0.04                           | AgBr-Cl  | 0.08                   |
| 3        | (II)            | 0.08                           | AgBr-Cl  | 0.03                   |
| 4        | (VI)*           | 0.04                           | AgBr-Cl  | 0.05                   |
| 5        | (III)           | 0.04                           | AgBr-Cl  | 0.04                   |
| 6        | (V)*            | 0.04                           | AgBr-Cl  | 0.08                   |

Sensitizing dyes (V) and (VI) have the following structures and were used for comparison:



What is claimed is:

1. A photographic silver halide emulsion containing a sensitizing dye represented by the general formula:



wherein each of groups V<sub>1</sub>, V<sub>2</sub>, W<sub>1</sub> and W<sub>2</sub>, which may be the same or different, represents a member selected from the group consisting of a hydrogen atom and a halogen atom, each of groups R<sub>1</sub> and R<sub>2</sub>, which may be the same or different, represents a lower alkyl group, A represents a member selected from the group con-

TABLE 3

| Test No. | Sensitizing dye | Amount (*) | Emulsion | Sensitization Maximum (m.μ.) | Sensitivity |
|----------|-----------------|------------|----------|------------------------------|-------------|
| 1        | (I)             | 0.09       | AgCl-Br  | 575-580                      | 950         |
| 2        | (II)            | 0.08       | AgCl-Br  | 574-578                      | 900         |
| 3        | (III)           | 0.04       | AgCl-Br  | 575-580                      | 950         |
| 4        | (I)             | 0.09       | AgBr-I   | 577-580                      | 980         |
| 5        | (II)            | 0.08       | AgBr-I   | 576-578                      | 950         |
| 6        | (III)           | 0.04       | AgBr-I   | 576-584                      | 1160        |

(\*): m. g. mol/kg. of emulsion

The sensitivity value was determined when the silver iodobromide emulsion was exposed through Fuji No. 3

sisting of a polymethylene group and an alkyl-polymethylene group, and n is an integer from 1 to 4.

2. A photographic silver halide emulsion as claimed in claim 1, wherein said sensitizing dye is



3. A photographic silver halide emulsion as claimed in claim 1, wherein said sensitizing dye is



4. A photographic silver halide emulsion as claimed in claim 1, wherein said sensitizing dye is



5. A photographic silver halide emulsion as claimed in claim 1, wherein said sensitizing dye is



\* \* \* \* \*

25

30

35

40

45

50

55

60

65